

# UNITED STATES PATENT OFFICE.

JOSEPH R. DRANEY, OF RIDGEWOOD, NEW JERSEY, ASSIGNOR, BY MESNE ASSIGNMENTS, TO BITOSLAG PAVING COMPANY, OF NEW YORK, N. Y., A CORPORATION OF DELAWARE.

## PAVING MIXTURE AND METHOD OF MAKING THE SAME.

1,364,621.

Specification of Letters Patent.

Patented Jan. 4, 1921.

No Drawing.

Application filed January 18, 1917. Serial No. 143,030.

To all whom it may concern:

Be it known that I, JOSEPH R. DRANEY, a citizen of the United States, residing at village of Ridgewood, in the county of 5 Bergen and State of New Jersey, have invented new and useful Improvements in Paving Mixtures and Methods of Making the Same, of which the following is a specification.

- 10 This invention relates to a pavement mixture as a product, the method of making the same, and also to the final roadway or pavement having its wearing surface constructed from the product.
- 15 The invention contemplates, broadly: (1) the method of making an improved paving mixture or product, which method or process consists, generally, in mixing with a mineral aggregate preferably of slag, a 20 portion of a suitable filler material, such as pulverized limestone, or other finely divided substance; mixing with a bitumen binding agent, which is preferably "blown" or oxidized asphalt, the remaining portion of the 25 filler material; and then admixing these two mixtures to form the final paving material; (2) a paving mixture resulting from the process above described and which is characterized by its homogeneity, density and 30 wearing qualities; and (3) a roadway or pavement which has the ability to withstand the wear of traffic to which it is subjected.

By proceeding in accordance with the method or process herein described, a paving 35 mixture is obtained in which the ingredients or materials are thoroughly and closely amalgamated; the binding agent is properly distributed throughout the mass, so that a homogeneous product is obtained in which 40 the pulverized material is thoroughly incorporated or impregnated with the bituminous binding agent; and the voids between the particles of mineral aggregate are filled to the desired percentage. The resultant 45 paving mixture is impervious to street acids or other moisture and has the attributes of great stability, and the capability of resisting deterioration under temperature changes or the strain of traffic to which it may be 50 subjected.

A roadway or pavement having its wearing surface constructed of the product above described is characterized by its wear-resisting qualities and by its ability to resist deterioration, crawling, creeping, undue def- 55 ormation, or fracture when subjected to traffic wear, or adverse moisture and heat conditions. It will be found that the wearing surface of the roadway has great dura- 60 bility, and sufficient rigidity to stand up under traffic strain, and yet it is sufficiently malleable or resilient to prevent chipping or breaking.

Having set forth the particular objects of my invention, I will now give the ma- 65 terials or ingredients which go to make up my new paving mixture, and describe in detail the steps employed in carrying out my improved method or process.

For the mineral aggregate, which is to 70 serve as the wear-resisting body of the pavement, I use slag which is obtained as a by-product of the blast furnace. The molten slag from the blast furnace is spread out and allowed to cool in the air so as to 75 permit it to weather in order that any soluble material may be leached out, and so that any shrinking, cracking or disintegration which is to take place will occur before the 80 slag is employed in the paving mixture. 80

Air-cooled blast-furnace slag is very hard in character, has great tensile strength, and will not chip, crack or break when subjected to ordinary traffic strains. The surfaces of the particles of slag are very rough, and 85 as they are irregular in shape and slightly porous, or to be more exact, cellular in make-up, the binding material used in the paving mixture may grip the particles of aggregate and hold them in position. The physi- 90 cal characteristics of slag are such that a very intimate binding of the slag aggregate and the binder will result, with, of course, less tendency to separation under traffic and greater stability and less likelihood of dis- 95 integration under temperature changes. Slag fracture is irregular and rough so that close union can be secured between the slag aggregate and the binder, and, furthermore, slag does not exhibit any appreciable 100

amount of dust. These are distinct advantages over stone aggregate, for stone fractures, comparatively speaking, are smooth and uniform and the surfaces present always a very considerable amount of dust, so that by reason of the smooth and dusty surfaces the stone does not give as satisfactory binding areas as does slag. This is true of the limestone and granite aggregates, the surfaces of which are smooth, carry a considerable amount of dust and, being non-porous or non-cellular, fail to afford the irregular gripping area found in slag.

Any suitable filler material, such as pulverized limestone or Portland cement, may be employed to fill the spaces or voids between the particles of the mineral aggregate, but preferably I use a filler of pulverized slag or slag dust. Due to the inherent cementitious properties of slag and its porosity cellular structure, the binding agent will adhere closely to the particles of slag-dust, and shifting of the fine particles of filler is guarded against.

As the bituminous binding agent, I employ "blown" or oxidized asphalt which may be produced very economically from heavy asphaltic base petroleums. It is found that "blown" or oxidized asphalt is less malleable than asphalt which is produced by other methods, but while its cementitious qualities are not as great as the usual distilled asphalt, yet it is characterized by its low susceptibility to moisture and temperature changes. Due to its rigidity, "blown" asphalt is particularly adapted for use in asphalt pavements for it has the necessary tensile strength to stand up under traffic strains without danger of disintegrating, and yet it possesses the necessary malleability or resiliency to resist cracking or chipping and, additionally, its element of rigidity is such that it maintains the particles of mineral aggregate and filler material against shifting.

Blown asphalt, as stated above, has not the high cementitious quality of distilled asphalt, for it becomes, by reason of oxidation, somewhat waxy in character and its content of oil is less than that of distilled asphalt. It will not, therefore, adhere as strongly to the relatively smooth dusty surfaces of stone aggregates and for that reason has by some been heretofore regarded as of little value in paving mixtures.

Combined, however, with slag, the properties of which have been heretofore pointed out, it produces a strongly adherent mixture, for notwithstanding its relatively low cementitious properties it grips and adheres tenaciously to the rough cellular slag fracture. Blown asphalt gives up its oil very slowly and it is, therefore, particularly well fitted for use with slag aggregate which, because of its cellular formation, is not par-

ticularly well adapted for use with the ordinary asphalt cement, the reason for this being that the continuous absorption of oil from the ordinary asphalt by the porous or cellular slag soon results in a deadening of the asphalt due to loss of oil and the disintegration of the asphalt binder.

The blown asphalt exhibits but little change under varying temperatures, and is, for that reason, more stable, and a pavement formed of a mixture in which blown asphalt or cement is used has greater and more uniform rigidity under all conditions, although it is resilient and malleable enough to be proof against chipping or fracture even under conditions of low temperature.

In carrying out my improved process or method, I first select hard, air-cooled, blast furnace slag, preferably weathered, as hereinbefore stated, and crush the same into small particles, so that the particles will pass through a screen of about one-fourth inch mesh. After careful screening, the slag mineral aggregate is graded into sizes so that, when mixed, the voids or spaces between the larger particles may be filled by the particles of the next smaller size, and the voids or spaces between the second size of particles are filled by the particles of the still smaller size, and so on down through the various gradations. The graded mineral aggregate is dried and heated preferably to a temperature between 350° and 450°, and while hot it is measured into a suitable mixing apparatus.

I next divide the filler material into two portions, one of the portions being, in weight, approximately equal to thirty-five (35) per cent. of the weight of the binding agent which is to be used in the mixture. The other portion of the filler or pulverized material is added to the graded and heated slag, the filler being added in a cold condition. The mineral aggregate and the added pulverized material are then mechanically mixed until uniform and the filler is properly distributed throughout the mass of the slag aggregate.

The asphalt composed of "blown" or oxidized heavy petroleum bases is then melted in a kettle and, while it is in molten condition, there is added thereto the remaining portion of filler dust or "fines," and, preferably, this portion of "fines" is equal to about 35% of the weight of the bituminous binding agent. The asphalt is maintained in molten condition and is thoroughly agitated by any suitable means, so as to thoroughly and uniformly distribute the "fines" throughout the mass of asphalt, and to keep the "fines" in suspension.

By mixing a portion of "fines," in substantially the amount specified, with the blown asphalt, a primed mixture is secured, and a very intimate relation results between

the asphalt and "fines," so that a very ready blending or mixing with the remaining filler and slag is secured.

Furthermore, this preliminary introduction of the "fines" into the blown asphalt takes up to a considerable extent the free oil and gives a mixture which is properly tempered for mixing with the remainder of the filler material and the aggregate.

10 The next step of my process consists in adding the "fines-impregnated" asphalt, in a molten condition, to the heated mixture of slag and filler material, which has been previously measured into the mixer. The 15 resultant mixture is then thoroughly agitated, so that the fines impregnated asphalt is thoroughly distributed throughout the mass. Upon continued stirring the surfaces of the particles of the mineral aggregate are properly coated with the asphalt, and the fines are thoroughly impregnated with the bitumen, so that a homogeneous and uniform paving mixture is obtained.

10 The paving material resulting from the 25 process above described is capable of taking care of a wide range of traffic conditions, and may be laid on any suitable foundation, such as a concrete base, old macadam, old brick pavements, or a layer of slag. After 30 mixing the mineral aggregate, "fines," and binding agent in the manner above described, the resultant paving mixture is placed in air tight vehicles and transported to the location of the work. On arriving 35 at the site, the mineral aggregate is dumped at a point sufficiently remote from its place of final deposition to allow all portions of the load being rehandled by the shovelers before final placing. It should be spread 40 to a uniform depth upon the foundation previously prepared and suitably rolled so that it will provide a compressed wearing surface.

I have found that by proceeding in accordance with the method above described, a final paving mixture results, in which the bituminous binding agent composed of "blown" asphalt is thoroughly distributed throughout the mass. The particles of 45 mineral aggregates are properly coated and the asphalt is so thoroughly incorporated with the pulverized material, that the interstices or pores of the pulverized material are filled and an intimate and close association 50 of the mineral aggregate and filler with the asphalt is obtained.

I am aware that it is broadly old to use slag in paving mixtures, but it is to be noted that, in the present instance, the slag is 60 employed in connection with "blown" or oxidized asphalt. As has previously been pointed out, "blown" asphalt has not the same cementitious properties as ordinary distilled asphalt, but its use is advantageous 65 over the use of distilled asphalt, in

that it is more rigid and less susceptible to heat changes and moisture. The deficiency in the cementitious character of the "blown" asphalt is, however, compensated for by the use of air-cooled blast furnace 70 slag. The slag with its natural rough cellular surfaces possesses inherent cementitious properties, so that after the pavement is laid a chemical change takes place in the slag, and a close chemical union is obtained 75 between the slag and the blown asphalt.

Furthermore, as the slag particles are irregular in shape and are characterized by their porosity or cellular structure, the asphalt when mixed with the slag will tend 80 to flow into the pores, and thus hair-like fingers are formed which grip the aggregate and hold it fast. As the "blown" asphalt is characterized by its rigidity, and the mineral aggregate of slag by its inherent 85 cementitious properties, irregular shape and porosity or cellular formation, there is present a very close bond or union between the particles of the aggregate and the "blown" asphalt. The "blown" asphalt tenaciously 90 grips the particles of slag, so that a very tough product is obtained. The mixture is very homogeneous and dense, and it is only slightly susceptible to temperature 95 changes and is characterized by its ability to resist street acids or other moisture.

A roadway formed with a wearing surface composed of my improved product is very durable, economical and non-slippery, and pleasing to the eye. It possesses low 100 susceptibility to temperature changes, great toughness, and sufficient rigidity to prevent creeping or deformation, and yet it is sufficiently elastic or resilient to prevent cracking or chipping.

#### What I claim is:—

1. The process of producing asphaltic paving material, which consists in mixing a portion of the filler material with a mineral aggregate of slag, mixing the remaining 110 portion of the filler material with the bituminous binding agent, and then admixing the two mixtures thus formed.

2. The process of producing asphaltic paving material, which consists in mixing 115 a portion of the filler material with a mineral aggregate of slag, mixing the remaining portion of the filler material with a bituminous binding agent of "blown" or oxidized asphalt, and then mixing the two 120 mixtures thus formed.

3. The process of producing asphaltic paving material, which consists in crushing the mineral aggregate composed of air-cooled blast furnace slag, grading the slag, 125 heating the slag, mixing with the heated and graded slag a portion of the pulverized filler material, heating the asphaltic binding agent to a molten mass, adding the remaining portion of the filler material to the 130

melted binding agent, and then admixing and thoroughly agitating the mixtures thus formed.

4. The process of producing asphaltic paving material, which consists in melting the bituminous binding agent, adding to the molten binding agent a portion of the "fines" equal to approximately 35% of the weight of the binding agent, mixing with a mineral aggregate of slag the remaining portion of the "fines," and then admixing the two mixtures thus formed.

5. The process of producing asphaltic paving material, which consists in melting a bituminous binding agent composed of "blown" or oxidized asphalt, adding to the molten asphalt a portion of the "fines" equal to approximately 35% of the weight of the asphalt, mixing with a mineral aggregate of slag the remaining portion of the "fines," and then admixing the two mixtures thus formed.

6. An asphaltic paving material consist-

ing of a mineral aggregate of slag, a suitable filler material, and a binding agent composed of "blown" or oxidized asphalt.

7. An asphaltic paving material consisting of a mineral aggregate of air-cooled blast-furnace slag, a pulverized material, and a binding agent composed of "blown" or oxidized asphalt.

8. An asphaltic paving material consisting of a mineral aggregate of air-cooled blast-furnace slag, a filler material composed of pulverized or dust-like slag, and a binding agent of "blown" or oxidized asphalt.

9. A roadway comprising a suitable foundation and a layer thereon formed of a mineral aggregate of slag, a filler of pulverized material, and a binding agent of "blown" or oxidized asphalt.

In testimony whereof I have hereunto set my hand.

JOSEPH R. DRANEY.